

Oct. 9, 1956

H. L. CROWLEY ET AL

2,766,117

PROCESS OF HEAT TREATING POWDERED METAL PARTS

Original Filed June 6, 1950

4 Sheets-Sheet 1

*Fig. 1*

*PRESSED AT 25,000 P.S.I.*



LEGEND:

- 10% HCl
- 5% HCl
- 2% HCl
- ◎ 1% HCl
- × 0.5% HCl
- 0% HCl

INVENTORS  
Henry L. Crowley  
By Marion Ernest Graham

Robert P. Dunham  
ATTORNEY

Oct. 9, 1956

H. L. CROWLEY ET AL

2,766,117

PROCESS OF HEAT TREATING POWDERED METAL PARTS

Original Filed June 6, 1950

4 Sheets-Sheet 2

Fig. 2

PRESSED AT 50,000 P.S.I.



LEGEND

- ◎ 15% HCl
- 10% HCl
- 5% HCl
- 2% HCl
- ◎ 1% HCl
- × 0.5% HCl
- 0% HCl

INVENTORS  
Henry L. Crowley  
Marion Ernest Graham  
BY

Robert P. Deubam

ATTORNEY

Oct. 9, 1956

H. L. CROWLEY ET AL

2,766,117

PROCESS OF HEAT TREATING POWDERED METAL PARTS

Original Filed June 6, 1950

4 Sheets-Sheet 3

Fig. 3

PRESSED AT 25,000 P.S.I.



INVENTORS  
Henry L. Crowley  
BY Marion Ernest Graham

Robert A. Deuker

ATTORNEY

Oct. 9, 1956

H. L. CROWLEY ET AL

2,766,117

PROCESS OF HEAT TREATING POWDERED METAL PARTS

Original Filed June 6, 1950

4 Sheets-Sheet 4



2,766,117

**PROCESS OF HEAT TREATING POWDERED METAL PARTS**

Henry L. Crowley, South Orange, N. J., and Marion Ernest Graham, Parma, Ohio, assignors to Republic Steel Corporation, Cleveland, Ohio, a corporation of New Jersey

Substituted for abandoned applications Serial No. 166,312, June 6, 1950, and Serial No. 300,908, July 25, 1952. This application April 3, 1956, Serial No. 575,794

17 Claims. (Cl. 75—224)

The present invention relates to a process of heat treating powdered metal parts and more particularly to heat treating and/or sintering such parts formed by pressing powdered metal into a desired shape in order that the parts as heat treated or sintered shall have desired physical characteristics.

As such the present application is a continuation-in-part of our prior and copending application Ser. No. 300,908, filed July 25, 1952, and now abandoned, and entitled, "Process of Heat Treating Powdered Metal Parts and Parts Formed Thereby"; said application Ser. No. 300,908 in turn being a continuation-in-part of our earlier application Ser. No. 166,312, filed June 6, 1950, and now abandoned. It is intended that the present application shall be a substitute for each of the earlier applications here identified.

In the past it has been customary in the making of parts by so-called "powder metallurgy" practices to select the powder of one or more metals, mix if powders of more than one metal are used, compact this powder in a suitable mold under relatively high pressure, then sinter the pressed parts in a non-oxidizing atmosphere at a suitable temperature, which is chosen in respect to the composition of the parts, in order that the metal powder shall be bound together into the desired article. Parts so formed are usually not as strong as a part made from cast metal, but they have the advantage that little or no machining need be done following the formation of the desired part in this way. As a result, the parts may be given adequate mechanical strength for some particular purposes, not requiring the strength of cast metal parts, and at the same time be made much quicker and cheaper. Such prior art processes have been applied using single metals and using combinations of metals, usually by mixing the powders of two or more metals in desired proportions. The atmospheres in which the heat treating or sintering has been done are uniformly non-oxidizing in character, but within that limitation, have been of many different types. All this prior art practice is now quite well known and is described in numerous text books on the subject.

The present invention improves this prior art practice in a substantial manner in that parts may be formed and heat treated in accordance with the present invention, so as to have greatly enhanced physical properties, for example, tensile strength, elongation and hardness, when heat treated at the same temperatures that would have been used in accordance with prior art practices. Alternatively, at least as good physical properties may be imparted to a given part as in the prior art, while using substantially lower temperatures for the heat treating than was thought possible in accordance with prior art practices. Intermediate results may be obtained in accordance with the present invention, including somewhat enhanced physical properties as aforesaid, while using somewhat

lower temperatures than were considered standard in accordance with the prior art teachings.

The present invention further improves on prior art practices in that by using the same conditions of temperature, the same results, or even better results, may be obtained in a shorter time period. Alternatively, the temperatures may be somewhat lower than have been standard in the prior art for various metal combinations respectively, and the same rate of production may be attained by resorting to the processes of the present invention. In other words, articles may be formed with the same or enhanced properties in respect to corresponding prior art articles, but in a shorter time and sometimes also at a lower temperature.

15 Summarizing the present invention, the processes in accordance therewith all involve heat treating in an atmosphere including gaseous hydrogen chloride. The improvements in the physical properties of the parts made according to the present process are more or less proportionate to the concentration of hydrogen chloride in the atmosphere about the parts during the heat treatment, in most instances up to about 10% to 15% hydrogen chloride concentration in this atmosphere by volume. For the purposes of the present invention, the minimum amount of 20 hydrogen chloride in the atmosphere may be taken to be about 0.1% gaseous hydrogen chloride by volume. The enhanced physical characteristics of the final product reach their peaks for most of the metals and combination thereof as hereinafter set forth at about 10% to about 25 15% by volume gaseous hydrogen chloride in the atmosphere, so that it is pointless to use any higher percentages; and in fact from some points of view, as hereinafter set forth, the use of higher concentrations of hydrogen chloride may be undesirable. It is found further that when the 30 gaseous atmosphere surrounding the part during the heat treating contains some reducing gas, as hydrogen, correspondingly better results are attained as compared to the use of a completely neutral gas, as nitrogen. The metals which are susceptible to forming into parts in accordance 35 with the present invention are broadly, the relatively difficultly chloridizable metals, namely, one or more metals selected from the group consisting of (a) the metals: iron, copper, nickel and cobalt and mixtures and alloys consisting essentially of at least two of said metals, (b) mixtures and alloys corresponding generally to bronze and consisting essentially of up to about 10% tin and the balance copper, (c) mixtures and alloys corresponding generally in composition to ferrous base alloys and consisting essentially of:

up to about 4% carbon,  
up to about 20% tungsten,  
up to about 1.75% manganese,  
up to about 28% chromium,  
up to about 8½% molybdenum,

50 and the balance in any such composition iron, whereon iron is present in a predominant amount.

Some relatively easily chloridizable materials do not lend themselves to treatment in any manner similar to 55 the present invention. Examples of such materials are zinc, aluminum, magnesium, titanium and alloys containing a substantial proportion of one or more of these metals. Such materials are to be considered as positively excluded from the scope of the appended claims.

60 Considering now details of the present invention and the principles governing it, there will be discussed first the metal or metals which may be used in accordance with this invention. Broadly, as aforesaid, the metals usable are practically restricted to those metals which are

relatively difficult to chloridize. The list of such appropriate metals and alloys is given above. This list includes all the metals now known to be usable, singly or in combination, in metal parts which may be processed in accordance with the present invention. In the event that some one of the relatively easily chloridizable metals, such as zinc, aluminum or magnesium, be present in any substantial amount, either alone, as an ingredient of a mixture, or as one metal forming an alloy with some other metal or metals which may be in the acceptable list given above, trouble is encountered. For example, brass, an alloy consisting of copper and zinc, is not to be considered as included in the purview of the processes set forth in the present claims; in contrast with this, bronze, consisting essentially of copper and up to 10% tin may be formed and heat treated in accordance with the present invention and within the scope of the appended claims. This will appear more particularly in examples hereinafter given.

The present invention is applicable when one or more metals are used, whether the metals, if two or more, be introduced as separate powders of the individual metals or as alloy powders, i. e.—wherein each particle of the powder is an alloy. When separate powders of individual metals are originally used in making the parts, there is considerable evidence that there is increased interdiffusion of the metal particles when operating in accordance with the process of the present invention as compared with prior art processes.

The theory, which is now believed to be basically correct, but is not particularly relied upon in support of the patentability of the appended claims, is that when substantial amounts of hydrogen chloride are present in the atmosphere during heat treating, relatively easily chloridizable metals are attacked by the hydrogen chloride to such an extent that the final product has present therein substantial amounts of the chlorides of the easily chloridizable metals and/or is porous due to the volatilization of such chlorides, leaving spaces formerly occupied by the chloridized metals. In either event, there results a product, different in composition from the metal powder which was subjected to the pressing operation and introduced into the heat treating step, which product has, in fact, less desirable physical characteristics than would be present if prior art practices were employed using a non-oxidizing atmosphere without hydrogen chloride present therein.

The next major factor to be considered in the present case is the atmosphere which is to be used during the heat treating. This atmosphere must be essentially non-oxidizing in character. It may be neutral or reducing, but cannot be to any substantial extent oxidizing. Many such atmospheres (absent hydrogen chloride) have been tried in the prior art, so that no particular details need be given here of the large number of different possible non-oxidizing atmospheres which are usable. It is found, however, in actual tests, as more particularly evident from examples given hereinafter, that nitrogen, a neutral gas, in operative as the non-oxidizing atmosphere. It has been found, however, that when the atmosphere surrounding the parts during the heat treatment used is reducing in character, such as a gas containing or consisting of hydrogen (other than the hydrogen chloride present therein), better results are obtained than with a strictly neutral gas. Thus, the preferred atmosphere, in accordance with the present invention, is one in which there is a substantial proportion of hydrogen. The theories now available tending to explain this will be stated hereinafter.

The essential distinction between the present invention and the prior art is in the use of some gaseous hydrogen chloride as a part of the atmosphere surrounding the metallic parts during the heat treatment thereof. It is found that when this process is carried on, the parts as finally made and as a result of the heat treatment, have enhanced physical characteristics of tensile strength and usually also of elongation, and to some extent also, hard-

ness, in respect to articles made in the same way throughout, with the exception that the atmosphere in which they are heat treated contained no hydrogen chloride. These differences will be apparent from particular examples hereinafter given and from the accompanying drawings.

The advantages to be gained by the presence of hydrogen chloride in the gases surrounding the articles in the heat treatment is more or less proportionate to the concentration of hydrogen chloride, in that greater advantages are gained in the case of most of the metals and alloys listed above by using higher percentages of hydrogen chloride until a concentration of (by volume) about 10% to about 15% hydrogen chloride is reached. At and beyond this range of concentrations, a plot of the value of certain physical characteristics against hydrogen chloride concentration levels off. Based upon plots of this kind, such as are shown in the accompanying drawings, it is the principle of this invention that any amount of hydrogen chloride is advantageous, so long as the hydrogen chloride is derived from a source separate and independent of the presence of any intermixed chlorides in the parts being treated, for example, when the hydrogen chloride is supplied as such in gaseous form to the gases, which are supplied from some external source to and/or are passed through the chloridizing zone. The same results cannot be obtained, however, by reliance upon the generation of hydrogen chloride in situ adjacent to the articles by supplying some chloride intermixed with the metal powder making up the articles being treated and by supplying some gaseous hydrogen in the atmosphere surrounding the articles for reaction with such intermixed chloride to produce hydrogen chloride, or even by supplying as an admixture in the articles a decomposable chloride, such as ammonium chloride, which may decompose under the temperature conditions present to give hydrogen chloride. It is believed that this is due to the fact that under such conditions voids are left in the metallic body being sintered which results in a decrease in the strength, which such articles would otherwise have. As hereinafter more particularly set out, when the amount of intermixed chloride is very small, the undesired results of its presence may be overcome by the enhanced and desired results due to the presence of sufficient, separately introduced hydrogen chloride in the gases, so that the final product will have properties superior to those of prior art articles.

In order that the present invention may be definite and easily understandable by those skilled in the art, an arbitrary value of 0.1% hydrogen chloride is hereby stated as the minimum hydrogen chloride concentration in the gas by volume which will be considered to be within the limits of this invention. A preferred range, however, of concentration of hydrogen chloride in accordance with the present invention is from about 0.5% to about 10% by volume. For maximum advantages from the point of view of physical characteristics of the final product, in accordance with the present invention, the range of about 5% to about 15% has been found to be preferred for most metals and combination thereof to which the invention is applicable. Beyond 15% there seems to be no purpose in increasing the hydrogen chloride concentration as the costs of the operation are increased to some extent and the physical properties of the final product, not substantially better. In addition to this, as the concentration of hydrogen chloride in the gases is raised, the tendency towards chloridizing some of the metal present is somewhat increased.

This point is related to the theories now believed to be correct for the use of an atmosphere containing some reducing gas, as hydrogen. Taking iron, for example, there is a progressively increasing tendency, as the hydrogen chloride concentration is increased, for a reaction to occur between the iron and hydrogen chloride to form ferrous chloride. If any ferrous chloride be formed,

even instantaneously, any hydrogen present in the gases will tend to reduce it to reform iron and to liberate hydrogen chloride in gaseous form. Thus, from an overall point of view, the presence of hydrogen in the atmosphere tends to prevent the formation and possibly the subsequent volatilization of ferrous chloride. Corresponding reactions can occur between other metals present and hydrogen chloride. For this reason, it is usually preferred to keep as low a hydrogen chloride concentration as possible, consistent with obtaining desired results, while at the same time having some hydrogen present in the gases. Another factor to be considered is the tendency for gases containing hydrogen chloride to corrode the apparatus in which the process is carried on. Here again, in order to minimize such corrosion, it is usually desirable to use as low a concentration of hydrogen chloride as can be used, while still obtaining the advantages of the present invention in producing articles having enhanced physical properties.

In contrast with the above, it is the present theory that when hydrogen chloride is used in accordance with the present invention in an atmosphere consisting, apart from hydrogen chloride, of a neutral gas such as nitrogen, there are opposing effects. The presence of hydrogen chloride will give enhanced physical characteristics in the final product in accordance with the present invention. On the other hand, the presence of hydrogen chloride, in the absence of a strongly reducing gas, such as hydrogen, will result in some chloridizing of the metal. This in turn will result in relatively less desirable physical properties. The net result, as will appear hereinafter from an actual example, is that physical properties somewhat enhanced in respect to those resulting from prior art practices are obtained when using hydrogen chloride and a neutral gas; but these properties are not as desirable respectively as are the properties of a corresponding article, heat treated in about the same concentration of hydrogen chloride in a gas also containing hydrogen. Preferably, however, the hydrogen concentration in a gaseous mixture including a neutral gas should be substantially equal to the proportion of hydrogen chloride therein.

Several theories have been formulated tending to explain the novel and highly beneficial results obtained from the practice of the present invention. One of these theories is that the hydrogen chloride present acts in a manner similar to a pickling bath, in that it serves to clean the surfaces of the metallic particles by removing any oxide film therefrom. This leaves the particles with clean surfaces, which are enabled more efficiently to sinter together, so as to form a superior article under a given set of conditions. The removal of the oxides thus results in enhanced physical characteristics for the final articles.

Another theory, which perhaps partakes of the above theory to some extent, is that the hydrogen chloride present in the gases reacts with any metallic oxides present to convert them to the respective chlorides. These chlorides, in a process in which the gases contain some hydrogen, may be reduced; and the reduced metal so formed may then act as a cement or binder to bind the particles of the original metallic material together. In such an event, the hydrogen chloride acts in effect as a catalyst, as it is regenerated by the reduction reaction with hydrogen.

Another theory which is in some respects related to the theory just explained is that hydrogen chloride may react with some of the finer of the metallic particles, converting them into the respective chlorides and generating hydrogen. Then some hydrogen, the same or some other hydrogen or both, present in the gases, may then react with the chlorides formed to regenerate the metals, but this time to deposit metal respectively so as to cement together or to increase the size of those particles and the bonds therebetween in a manner similar to that in which crystals grow in a solution. In such an event also the hydrogen chloride acts in effect as a catalyst, as it is regenerated and not consumed to a substantial extent.

While the theories expressed herein are now believed to be correct, the patentability of the appended claims is not predicated upon the correctness of these theories, or any of them, but rather upon the novel combination of process steps specifically recited herein. It is not known exactly why these improved results occur. It is known, however, that they do in fact occur and that they are reproducible when the teachings of this application are followed.

- 10 It appears that the hydrogen chloride must be present in gaseous form in the atmosphere surrounding the articles, and that this gaseous hydrogen chloride must be obtained at least in a large part from some one or more sources other than decomposition of a chloride introduced 15 in admixture with the metallic material, or resulting from a reaction between such intermixed chloride and any hydrogen in the gaseous atmosphere. This was proven by the fact that while gaseous hydrogen chloride was effective in securing enhanced physical properties in an iron body or article, no correspondingly desirable results were attained when using an atmosphere as in the prior art including hydrogen and when chloride was supplied in the form of solid ferrous chloride intermixed with the iron powder as a part of the article to be heat treated. 20 25 This was so even though the atmosphere used surrounding the ferrous chloride-containing-article consisted solely of hydrogen. This result was surprising in view of the fact that it is known that in an atmosphere of hydrogen, ferrous chloride is largely reduced to metallic iron at the 30 temperature and in the time at which these articles were held for heat treatment. Under the circumstances of the test, wherein the powdered iron article contained a relatively large amount of solid  $FeCl_2$ , the article produced had a lower physical strength as compared with an article 35 formed of pure iron powder and heat treated in accordance with the prior art at the same temperature. From this it was concluded that in order to attain the desired results of the present process, it is not feasible to supply chloride as solid ferrous chloride intermixed in the article itself, so that hydrogen chloride must be otherwise supplied to or be present in the gases surrounding the article during the heat treatment.

As hereinafter set forth by examples which follow, a very small amount of intermixed chloride, for instance 45 an amount in the order of magnitude of 0.1% to 0.25% by weight, will have such a small undesired effect upon the tensile strength of the final article that when such an article is sintered in an atmosphere containing hydrogen chloride from an external source, in accordance with the 50 present invention, quite desirable results are obtained. When the percentage of the intermixed chloride is as high as about 0.25, the undesired results thereof begin to be substantially felt. Progressively greater amounts of intermixed chloride give progressively worse results in terms 55 of the tensile strength of the final article. There is a point at which the desired results of the use of separately introduced hydrogen chloride in the gases will not serve to overcome the undesired results of intermixed chlorides in the original article. When greater amounts of intermixed chloride than this amount, to balance the desired results of hydrogen chloride, are present, the net effect of both on the tensile strength of the finished article is undesired in respect to following prior art practices. The preferred situation, therefore, is one in which the metallic 60 material formed into the articles to be sintered is free, or substantially free, of any intermixed chloride, as under these circumstances there is no, or substantially no, undesired effect therefrom, so that the desired effect of the presence of hydrogen chloride in the gases is not diminished by this opposing effect.

The next major factor to be considered in the present process is the temperature at which the heat treating takes place. In accordance with the prior art wherein the gaseous atmosphere did not contain hydrogen chloride, such temperatures were in fact standard, or substantially

so, for any given metal or combination of metals. For example, with powdered iron, the temperature used was about 2000° F. This standard temperature, chosen in accordance with the prior art, may be defined as that at which at least one metal present is brought to the point of incipient fusion. At the same time, these standard temperatures were always less than the melting point of the highest melting metal present. As such, therefore, the temperatures varied substantially depending upon the composition of the metal or metals contained in the part being heat treated. For the purpose of the present discussion, these prior art sintering temperatures in an atmosphere in which hydrogen chloride was absent may be termed standard temperatures. Such standard temperatures may be found in many text books and articles treating this subject matter.

In accordance with the present invention the process may be practiced at the standard temperature as aforesaid for the material in question and thereby greatly enhanced physical characteristics obtained in the final article, particularly tensile strength, and elongation, and to some extent also hardness. This practice may be termed one phase or embodiment of the present invention.

Another phase or embodiment of the present invention is to conduct the sintering operation at substantially reduced temperatures in respect to standard temperatures as aforesaid respectively. At such reduced temperatures, which are substantially less than the standard temperatures for any given metal composition, at least as great or as desirable physical properties may be attained in the final product as would result from the practice of prior art processes with respect to the same type article. For example, taking the case of an iron article, the standard temperature of the prior art is about 2000° F. when using an atmosphere containing no hydrogen chloride. In accordance with the present invention, a final article formed from iron powder can be prepared using a sintering temperature of about 1600° F. and having at least as desirable physical properties of strength and elongation. Thus, in accordance with this embodiment of the process of the invention, substantially less heat is required, with a corresponding saving in the cost of the heat and in wear and tear on the equipment used incident to the use of higher temperatures.

Intermediate practices may also be used in accordance with the present invention using temperatures between the standard temperature and the lowest temperature possible as aforesaid, which may be expressed as somewhat lower than the standard temperatures, and attaining results somewhat more desirable than those attainable in accordance with prior art practices.

It is also contemplated in accordance with the present invention, that a temperature may be used, when heat treating a metallic article including two or more metals, which temperature will be below the melting point of the highest melting metal present, but not necessarily below the melting point of one or more lower melting metals present. Using this phase of the invention, some one or more of the lower melting metals may, in fact, be caused to fuse, thus serving to bind together the unfused particles of the higher melting metal.

Another phase or embodiment of the present invention is that by employing an atmosphere including hydrogen chloride, in accordance with this invention, desired results at a given temperature may be obtained in a somewhat less time than was required when operating in accordance with prior art practices, wherein no hydrogen chloride was present in the atmosphere. Thus, for a given temperature, and as the time period for the sintering of a given article may be shortened by following the practice of the present invention, a given piece of equipment will have increased productivity in any time period, such as a day or a week. This desired shortening of the sintering time may be effective to render the process more desirable from an economic point of view and

may be balanced in part, at least, for example, by lowering the temperature somewhat, so as to save some heat formerly required, while still keeping the temperature high enough to give enhanced physical properties in respect to the prior art practices and while using a sintering time somewhat shorter than was considered essential in accordance with the prior art practices. Different combinations of these several variables as herein taught may be employed within the purview of the present invention.

In the accompanying drawings there are illustrated graphically some of the desirable results of the present invention, so that these results may be visualized more easily than could be done from mere tabulated results.

15 In the drawings:

Figure 1 is a plot showing the relation between the tensile strength and sintering temperature in iron articles previously pressed at 25,000 p. s. i. and with different concentrations of hydrogen chloride present in the atmosphere during the sintering;

Fig. 2 is a plot similar to Fig. 1, but with the articles pressed at 50,000 p. s. i.;

25 Fig. 3 is a plot showing the relationship between tensile strength and the concentration of hydrogen chloride present in the gaseous atmosphere during sintering, curves being shown for different temperatures, the material used being iron powder pressed at 25,000 p. s. i.; and

20 Fig. 4 is a plot similar to Fig. 3, but with the articles pressed at 50,000 p. s. i. rather than 25,000 p. s. i.

30 In each of the plots shown in the accompanying drawings, a comparison is given with the prior art, which is that condition represented by 0% hydrogen chloride. It will be noted from the several plots that substantially enhanced results as to tensile strength are obtained when 35 progressively greater concentrations of hydrogen chloride are present in the gases up to about 10%; and that these results are different to a substantial and surprising extent from those obtainable using prior art practices. While the data forming the bases for the curves shown in the 40 drawings was obtained using powdered iron test pieces, similar results are obtainable using other metals or combinations as set forth herein.

The data illustrated in Figs. 1 through 4 is set forth in tabular form in Tables 1 and 2 below. The Rockwell 45 hardness values referred to in Table 2 were obtained using a standard Rockwell test apparatus employing a  $\frac{1}{8}$ " steel ball and a 60 kilogram major load. All readings given are "H" scale readings.

50 TABLE I  
Iron powder pressed at 25,000 p. s. i. before heat treatment

| 55 | Percent HCl in Atmosphere | Temperature, °F. | Tensile Strength, p. s. i. | Elongation, Percent |
|----|---------------------------|------------------|----------------------------|---------------------|
| 60 | 0                         | 1,200            | 270                        | 0.2                 |
|    | 0.5                       | 1,200            | 370                        | 0.2                 |
|    | 1.0                       | 1,200            | 310                        | 0.5                 |
|    | 2.0                       | 1,200            | 680                        | 1.5                 |
|    | 5.0                       | 1,200            | 900                        | 0.8                 |
|    | 10.0                      | 1,200            | 1,330                      | 0.8                 |
|    | 10.0                      | 1,400            | 4,360                      | 1.9                 |
|    | 0                         | 1,600            | 5,760                      | 1.0                 |
|    | 0.5                       | 1,600            | 5,160                      | 1.3                 |
|    | 1.0                       | 1,600            | 5,680                      | 2.1                 |
| 65 | 2.0                       | 1,600            | 6,080                      | 2.3                 |
|    | 5.0                       | 1,600            | 6,640                      | 3.7                 |
|    | 10.0                      | 1,600            | 8,330                      | 4.7                 |
|    | 0                         | 1,800            | 6,580                      | 1.1                 |
|    | 0.5                       | 1,800            | 5,960                      | 1.7                 |
|    | 1.0                       | 1,800            | 6,540                      | 2.1                 |
|    | 2.0                       | 1,800            | 7,420                      | 3.1                 |
|    | 5.0                       | 1,800            | 8,590                      | 3.2                 |
|    | 10.0                      | 1,800            | 9,260                      | 4.6                 |
|    | 0                         | 2,000            | 7,260                      | 2.6                 |
| 70 | 0.5                       | 2,000            | 7,560                      | 2.4                 |
|    | 1.0                       | 2,000            | 7,760                      | 2.9                 |
|    | 2.0                       | 2,000            | 7,510                      | 2.4                 |
|    | 5.0                       | 2,000            | 9,160                      | 3.9                 |
|    | 10.0                      | 2,000            | 11,540                     | 5.3                 |

TABLE 2

Iron powder pressed at 50,000 p. s. i. before heat treatment

| Percent HCl in Atmosphere | Temperature, °F. | Tensile Strength in p. s. i. | Elongation, in Percent | R. C. |
|---------------------------|------------------|------------------------------|------------------------|-------|
| 0                         | 1,200            | 830                          | 0.3                    |       |
| 0.5                       | 1,200            | 1,240                        | 0.8                    |       |
| 1.0                       | 1,200            | 1,480                        | 1.1                    |       |
| 2.0                       | 1,200            | 1,250                        | 0.9                    |       |
| 5.0                       | 1,200            | 1,980                        | 1.0                    |       |
| 10.0                      | 1,200            | 2,960                        | 1.1                    |       |
| 10.0                      | 1,400            | 8,830                        | 2.8                    |       |
| 0                         | 1,600            | 10,080                       | 1.6                    | 50.8  |
| 0.5                       | 1,600            | 11,190                       | 3.1                    |       |
| 1.0                       | 1,600            | 10,800                       | 3.1                    |       |
| 2.0                       | 1,600            | 10,700                       | 3.6                    |       |
| 5.0                       | 1,600            | 12,400                       | 4.7                    |       |
| 10.0                      | 1,600            | 14,110                       | 6.2                    | 53.4  |
| 15.0                      | 1,600            | 14,560                       | 5.4                    |       |
| 0                         | 1,800            | 11,230                       | 3.1                    |       |
| 0.5                       | 1,800            | 11,970                       | 2.8                    |       |
| 1.0                       | 1,800            | 12,620                       | 3.4                    |       |
| 2.0                       | 1,800            | 12,970                       | 3.4                    |       |
| 5.0                       | 1,800            | 15,530                       | 3.7                    |       |
| 10.0                      | 1,800            | 15,640                       | 5.8                    |       |
| 0                         | 2,000            | 13,300                       | 3.4                    | 61.8  |
| 0.5                       | 2,000            | 13,640                       | 3.9                    |       |
| 1.0                       | 2,000            | 13,350                       | 4.2                    |       |
| 2.0                       | 2,000            | 15,230                       | 5.2                    |       |
| 5.0                       | 2,000            | 16,550                       | 5.2                    |       |
| 10.0                      | 2,000            | 17,680                       | 7.4                    | 65.3  |
| 15.0                      | 2,000            | 17,650                       | 7.5                    |       |

From Tables 1 and 2 above, it will be noted that the results obtained in terms of tensile strength and elongation for the tests made using lower concentrations of hydrogen chloride are somewhat spotty and irregular. Nevertheless, it is believed that desirable results may and often will be obtained, at least as to certain of the physical characteristics, even with relatively low concentrations of hydrogen chloride. On the other hand, it will be obvious from the tabulated data given above, that the preferred concentrations are the relatively higher ones, approaching 10%, at which positively improved results are always obtained in respect to prior art practices wherein no hydrogen chloride was used.

Additional tests were made on this same type of iron, as set forth in Tables 1 and 2 above, and at both 1600° F. and 2000° F., with the parts pressed at 50,000 p. s. i. as in Table 2 above, the percentage hydrogen chloride in the sintering gases being increased in these several tests to include the values of 15%, 30%, 50%, 75% and 100% hydrogen chloride with the balance (if any), hydrogen. The values of tensile strength were approximately constant within the limits of experimental error, and increased but slightly up to 100% hydrogen chloride, the value of the tensile strength at 100% hydrogen chloride, at 2000° F., averaging 17,920 p. s. i. From the above, it is concluded that concentrations of hydrogen chloride in excess of about 15% do not give any substantial increase in the tensile strength of the finished articles.

The application of the process of the invention to powdered metals other than iron may be illustrated by the following examples:

*Example 1.*—Powdered metal parts consisting of 92.5% iron powder and 7.5% copper powder by weight were produced by mixing copper and iron powders in these proportions and pressing the mixed powders to shape at 50,000 p. s. i. Some of these parts were then sintered in a pure hydrogen atmosphere at 1800° F. for one hour. Others of these parts produced under the same conditions were sintered for the same time and at the same temperature in an atmosphere consisting of 90% hydrogen and 10% hydrogen chloride gas by volume. The tensile strength of the part sintered in pure hydrogen was 16,000 p. s. i., these parts having an elongation of 1.5%. The corresponding parts that were sintered in the atmosphere containing 10% hydrogen chloride had a tensile strength of 22,230 p. s. i. and an elongation of 1.5%. This illustrates that sintering in atmospheres containing hydrogen

chloride has a beneficial effect on the tensile strength of copper-iron mixed powders.

*Example 2.*—Metal parts were prepared by mixing 97% of iron powder and 3% of nickel powder by weight and pressing the mixed powders at 50,000 p. s. i. Some of these parts were sintered for 1 hour in an atmosphere of pure hydrogen at 1800° F., while others, having the same composition, were sintered under the same conditions of time and temperature in an atmosphere consisting of 90% hydrogen and 10% hydrogen chloride gas by volume. The parts sintered in pure hydrogen had a tensile strength of 11,280 p. s. i. and an elongation of 3.1%; while other parts of the same composition sintered in the atmosphere containing hydrogen chloride had a tensile strength of 13,720 p. s. i. and an elongation of 4.2%.

Parallel tests were also run on powdered metal parts which were prepared in the same way, but which consisted of 94% iron and 6% nickel by weight. Of these samples, the ones sintered in a pure hydrogen atmosphere had a tensile strength of 11,980 p. s. i. and an elongation of 3.2%; while those that were sintered in an atmosphere consisting of 90% hydrogen and 10% hydrogen chloride by volume had a tensile strength of 14,450 p. s. i. and an elongation of 3.4%. Here again, the advantageous results of sintering in an atmosphere containing hydrogen chloride gas are demonstrated by an increase in tensile strength of the order of 20%, while there is also an increase in percentage elongation.

*Example 3.*—Powdered metal parts (simulating bronze), consisting of 90% copper powder and 10% tin powder were prepared by mixing these two powders and pressing the mixed powders to a desired shape at 50,000 p. s. i. Some of these parts were sintered for one hour in an atmosphere of pure hydrogen at a temperature of 1475° F.; while others were sintered under the same conditions in an atmosphere consisting of 90% hydrogen and 10% hydrogen chloride gas by volume. Those parts sintered in pure hydrogen had a tensile strength of 14,040 p. s. i. and an elongation of 0%; while those sintered in the atmosphere including hydrogen chloride gas had a tensile strength of 29,500 p. s. i. and an elongation of 8.6%. In this mixture, particularly, the advantages of sintering in hydrogen chloride-containing atmospheres are strikingly illustrated.

*Example 4.*—As an example of the application of the invention to gases of a non-reducing, neutral character, the results of sintering powdered iron parts in a nitrogen atmosphere are set forth below. Samples were prepared from the same type of powdered iron employed in the tests, the results of which are shown in Figures 1 through 4 and are set out in Tables 1 and 2 above, by pressing the iron powder to a desired shape at 50,000 p. s. i. Some of the test pieces so prepared were sintered for one hour at 1800° F. in an atmosphere of pure nitrogen, while others were sintered under the same conditions in an atmosphere consisting of 90% nitrogen and 10% hydrogen chloride gas by volume. Those test pieces sintered in the atmosphere of pure nitrogen had an average tensile strength of 11,130 p. s. i. and an average elongation of 0.9%; while those sintered in the atmosphere containing hydrogen chloride had an average tensile strength of 14,320 p. s. i. and an average elongation of 2.1%. Thus, it will be seen that when using a neutral atmosphere, such as nitrogen, the addition of hydrogen chloride enhances the physical properties of heat treated powdered metal parts. However, it will be noted by comparison with the data set forth in Table 2, that this increase of tensile strength is not as great as when the heat treatment is carried out in an atmosphere containing hydrogen.

During the tests on the heat treatment of iron articles in an atmosphere of nitrogen and hydrogen chloride, the presence of  $FeCl_2$  was observed in the exit gases. It is believed that during such a process the beneficial effects of the hydrogen chloride were partially counteracted by the formation and subsequent volatilization of  $FeCl_2$ .

which weakened the product physically to some extent. However, this undesired chloridization did not take place to such an extent as to prevent the hydrogen chloride from enhancing the tensile strength of the parts in respect to that of parts sintered in an atmosphere containing no hydrogen chloride. This example thus further illustrates the beneficial effects of the presence of a reducing gas, as hydrogen.

A further series of tests was conducted upon some nitrogen and varying amounts of hydrogen and hydrogen chloride. It was found that the best values of tensile strength were obtained when approximately equal concentrations of hydrogen and hydrogen chloride were present along with nitrogen, and that the requirements for hydrogen chloride in the gases in order to obtain maximum tensile strength indicated that products having increased tensile strength would be obtained up to about 10% hydrogen chloride. Thus, substantially the optimum conditions are reached with a gas concentration (by volume) of 10% hydrogen chloride, 10% hydrogen and 80% nitrogen giving a tensile strength for iron parts comparable to the tests set forth in Table 2 above (iron powder pressed at 50,000 p. s. i. and sintered at 2000° F.) of 17,260 p. s. i. With 30% hydrogen, 30% hydrogen chloride and 40% nitrogen, tensile strength averages 18,950 p. s. i.; while with 30% hydrogen chloride, 60% hydrogen and 10% nitrogen, tensile strength averages 18,980 p. s. i.

From the above, it will be seen that little increase in tensile strength of the finished parts is attained by using more than about 10% hydrogen chloride. Furthermore, these tests have shown that when less than about the equivalent amount of hydrogen in respect to hydrogen chloride is used, relatively lesser tensile strengths are obtained as set forth above. It is believed that the optimum conditions, therefore, are reached when substantially equal amounts of hydrogen and hydrogen chloride are used with some neutral gas, such as nitrogen, making up the gaseous atmosphere.

*Example 5.*—This example illustrates an attempt to apply the method of the present application to a pre-alloyed brass powder consisting essentially of 90% copper and 10% zinc by weight. As zinc is a metal which is relatively easy to chloridize, as compared with other metals included in the scope of the present invention, it was not expected that the process of the present invention would be applicable without change to any metallic material containing a substantial amount of zinc. This expectation was proved accurate by the tests made in accordance with this example. Test samples were prepared from the brass alloy powder described above, by pressing at 50,000 p. s. i. Some of the samples so made were sintered for one hour in an atmosphere of pure hydrogen at 1620° F., while others were sintered under the same conditions in an atmosphere consisting of 90% hydrogen and 10% hydrogen chloride gas by volume. The parts sintered in the atmosphere of pure hydrogen had a tensile strength of 10,150 p. s. i., and an elongation of 3.6%; while those sintered in the hydrogen chloride-containing atmosphere had a tensile strength of only 7,180 p. s. i. and an elongation of only 1.5%.

The decrease in tensile strength and percentage elongation, which was found when the process of the present application was applied to these parts, is believed to be attributable to the fact that the relatively reactive zinc-containing powder combines with the hydrogen chloride gas to form zinc chloride, which volatilizes at the temperatures employed, leaving the remaining structure of the part substantially weakened. As such, therefore, the general teachings of the present invention are not applicable to zinc-containing powders or parts.

*Example 6.*—The presence of solid chloride in admixture with a powdered metal part exerts an undesirable influence upon the resulting tensile strength of the part. This matter has been investigated from various points of view, the investigation in accordance with the tests

herein reported on using iron powder and anhydrous ferrous chloride, as an example of a chloride, so that reaction between ferrous chloride and hydrogen in the gaseous atmosphere would provide the same metal of which the part was made. Several samples were prepared by incorporating and intermixing various proportions of solid anhydrous  $FeCl_2$  with the powdered iron part being treated. The results of this series of tests (in which the parts were exposed to an atmosphere consisting essentially of hydrogen and wherein hydrogen was a still atmosphere, no attempt was made to circulate the hydrogen past the articles during the heat treatment, so as to permit the building of a hydrogen chloride concentration, if such were reasonably possible) are set forth in Tables 3 and 4 hereinafter given.

TABLE 3  
Iron powder pressed at 25,000 p. s. i. before heat treatment

| Percent Solid $FeCl_2$ in Mixture | Temperature, ° F. | Tensile Strength, p. s. i. | Elongation in Percent |
|-----------------------------------|-------------------|----------------------------|-----------------------|
| 0                                 | 1,800             | 6,580                      | 1.1                   |
| 0.25                              | 1,800             | 5,050                      | 1.5                   |
| 0.5                               | 1,800             | 5,370                      | 1.5                   |
| 1.0                               | 1,800             | 5,280                      | 1.5                   |

TABLE 4  
Iron powder pressed at 50,000 p. s. i. before heat treatment

| Percent Solid $FeCl_2$ in Mixture | Temperature, ° F. | Tensile Strength, p. s. i. | Elongation in Percent |
|-----------------------------------|-------------------|----------------------------|-----------------------|
| 0                                 | 1,800             | 13,940                     | 2.2                   |
| 0.25                              | 1,800             | 12,670                     | 1.6                   |
| 0.5                               | 1,800             | 13,550                     | 2.7                   |
| 1.0                               | 1,800             | 10,490                     | 2.4                   |

From the data given in Tables 3 and 4, it will be seen that while certain of the results are somewhat irregular, the general effect is a decreased tensile strength with increasing amounts of admixed ferrous chloride. Thus, the preferable condition is one in which there is no admixed chloride of any kind whatsoever in the part, with the possible exception of trace amounts present as impurities.

It has also been found that the presence of ferrous chloride in admixture with a powdered iron part has an effect which is variable, depending upon the time and conditions of exposure of the part to the atmosphere (based on the water vapor content thereof) between the admixing of the powder and pressing operation on the one hand, and the sintering operation on the other. This is believed to be due to the fact that anhydrous ferrous chloride tends to take up water from the atmosphere, probably forming some one or more of the hydrated ferrous chlorides; and that this tendency is not wholly prevented even though parts are kept in a desiccator during the interval between pressing and sintering. As a result, it has been found that when a substantial interval, such as a day or two, intervenes between the pressing and the subsequent sintering of the parts, and even if the parts after pressing are stored in a desiccator, such parts have irregular and relatively undesirable strength characteristics, as measured by the tensile strength of the final products.

When parts were formed as aforesaid, having but a very small amount of admixed ferrous chloride therein; and when these parts were sintered within not over ten minutes from the time of pressing to the time of introduction into the sintering oven, and when the sintering took place in the presence of hydrogen chloride gas derived from a source independent of the admixed ferrous chloride, the undesired effect of the admixed ferrous chloride, was offset by the desired effect of the practice

of the present invention. Thus, in a series of parts tested in this way, including  $\frac{1}{4}\%$  ferrous chloride in admixture with iron powder sintered in an atmosphere of 5% and 10% hydrogen chloride (the balance hydrogen), and when the gases were caused to flow past articles during the sintering operation, so as to maintain stabilized conditions, the following tensile strengths were found:

| Percent HCl in the Sintering Gas | Tensile Strength in p. s. i. |
|----------------------------------|------------------------------|
| 0.....                           | 7,800                        |
| 5.....                           | 12,600                       |
| 10.....                          | 13,800                       |

These results may be compared with a set of similar samples containing 0%  $\text{FeCl}_2$  and tested in the same way, which are as follows:

| Percent HCl in the Sintering Gas | Tensile Strength in p. s. i. |
|----------------------------------|------------------------------|
| 0.....                           | 7,800                        |
| 5.....                           | 13,600                       |
| 10.....                          | 16,400                       |

From the above, it will be noted that the tensile strengths resulting from the tests using 5% and 10% hydrogen chloride in the gases are better than when no hydrogen chloride is present. More desirable results are obtained, however, when from 5% to 10% hydrogen chloride is used. On the other hand, the tensile strengths of the parts having  $\frac{1}{4}\%$   $\text{FeCl}_2$  are respectively lower than those of the parts containing no admixed  $\text{FeCl}_2$ .

It is believed, therefore, that the presence of admixed chloride introduces an undesired effect which may be partly or wholly offset by the desired change or effect due to sintering the part in an atmosphere containing hydrogen chloride derived from a source separate and independent of the reaction between hydrogen present in the gases with admixed  $\text{FeCl}_2$ ; and that this is true irrespective of the presence of hydrogen in the sintering gas. It is, of course, possible that the undesired effects resulting from the presence of admixed ferrous chloride or other chloride will be so great as wholly to negative the desired result from the use of the hydrogen chloride containing atmosphere in accordance with the present invention, so that the net effect may be a poorer product than if neither were used or present.

It is preferable, therefore to minimize and more preferable to reduce to zero the amount of admixed ferrous chloride in accordance with the present invention, so as to realize to a maximum extent the desired results of the present process.

*Example 7.*—This example is to illustrate the application of the present process to articles made from nickel powder. Parts were prepared of nickel powder by pressing this powder at 30,000 p. s. i. (all that was required for a reasonably dense green compact) and then sintering at 2000° F. Different samples were sintered with gases having different hydrogen chloride (HCl) concentrations as set forth hereinafter. A sample of nickel prepared as aforesaid and which was sintered in an atmosphere of pure hydrogen had a tensile strength of 7,930 p. s. i. and an elongation of 4%. Another sample sintered in an atmosphere including 1% (by volume) hydrogen chloride and the balance hydrogen had a tensile strength of 8,520 p. s. i. and an elongation of 4.0%; while a sample which was sintered in an atmosphere consisting essentially of 10% hydrogen chloride and the balance hydrogen had a tensile strength of 11,390 p. s. i. and an elongation of 4.7%.

From the above it will be noted that when the process of the present invention was used, there was a substantial

(and in the case of 10% HCl, a very material) increase in tensile strength and a certain amount of increase in elongation.

*Example 8.*—Tests were made of the applicability of the present invention to parts made of 100% copper. In this instance copper powder was compacted at 20,000 p. s. i. and sintered at 1400° F., these values being found to be applicable in the case of copper. A group of samples was tested after being sintered in different gaseous compositions, i. e. compositions including different concentrations of hydrogen chloride, with the balance hydrogen in each instance. The test results showed that when sintered in an atmosphere of pure hydrogen, the parts had an average tensile strength of about 12,000 p. s. i. and an average elongation of about 6.7%; when sintered in an atmosphere consisting essentially of 1% hydrogen chloride and the balance hydrogen, the parts had an average tensile strength of about 12,900 p. s. i. and the same average elongation, i. e. 6.7%; while when sintered in an atmosphere of about 10% hydrogen chloride and the balance hydrogen, the parts had a tensile strength of about 17,050 p. s. i. and an average elongation of about 9.4%. This is deemed to show that the use of the process of the present invention with parts made of copper powder positively increases the tensile strength of the parts by very substantial amounts and increases the elongation somewhat, but again a substantial amount.

*Example 9.*—Parts were prepared using metallic cobalt powder 300-mesh size and made up using a pressing pressure of 60,000 p. s. i. and were later sintered at 2000° F. The tensile strengths of parts made using different amounts of hydrogen chloride mixed with hydrogen, were as follows:

| Percent HCl During Sintering | Tensile Strength in p. s. i. |
|------------------------------|------------------------------|
| 0.....                       | 64,700                       |
| 1.....                       | 72,300                       |
| 5.....                       | 71,200                       |
| 10.....                      | 66,800                       |

This indicates that the maximum strength as to articles of substantially pure cobalt is attained at a value between 1% and 5% (by volume) hydrogen chloride, the tensile strength falling off somewhat at 10%, but still being greater than that when no hydrogen chloride is used.

*Example 10.*—Parts were prepared using about 5% cobalt powder as in Example 9 above, and about 95% Swedish iron powder, the parts being pressed at 60,000 p. s. i. and later sintered in a gas consisting essentially of various percentages (by volume) hydrogen chloride and the balance hydrogen, at 2000° F. The results of these tests are shown in the following table:

| Percent HCl in the Sintering Gas | Tensile Strength in p. s. i. |
|----------------------------------|------------------------------|
| 0.....                           | 12,000                       |
| 1.....                           | 15,500                       |
| 5.....                           | 18,800                       |
| 10.....                          | 19,300                       |

Thus, when cobalt is mixed with iron, the results attained are progressively more desirable as the percentage of hydrogen chloride in the atmosphere is increased up to about 10%. This tensile strength value levels off, however, at about 10%, so that further increases in the hydrogen chloride concentration serve little useful purpose.

*Example 11.*—Parts were prepared using 5% tungsten and 95% Swedish iron powder; the parts being pressed at 50,000 p. s. i. and later sintered in a gas consisting essentially of various percentages (by volume) hydrogen

chloride and the balance hydrogen, at 2000° F. The results are shown in the following table:

| Percent HCl in the Sintering Gas | Tensile Strength in p. s. i. |
|----------------------------------|------------------------------|
| 0                                | 5,700                        |
| 1                                | 11,700                       |
| 5                                | 12,000                       |
| 10                               | 13,100                       |

Similar tests were made using about 10% tungsten with the balance iron. In these tests, a group of test bars was made of this composition and sintered in pure hydrogen. The average tensile strength of these bars was 7,950 p. s. i. and the average elongation, 3.0%. Another group of test bars of the same composition (about 10% tungsten with the balance iron) was prepared and sintered in a gaseous mixture consisting essentially of about 5% hydrogen chloride and the balance hydrogen. These bars showed upon testing an average tensile strength of 14,400 p. s. i. and an elongation of 4.5%. This shows a definite increase in tensile strength and in elongation respectively for the bars which were sintered in accordance with the present invention.

Another similar group of test bars was prepared and tested, the composition of which consisted essentially of about 20% tungsten and the balance iron. A group of these test bars was sintered in pure hydrogen and then tested with the results: tensile strength (average) 6,600 p. s. i., elongation (average) 2.4%. A further group of test bars made up in the same way and of the same composition (about 20% tungsten and the balance iron) was sintered in an atmosphere consisting essentially of about 5% hydrogen chloride and the balance hydrogen, and then tested as before. The average tensile strength of these bars was 16,370 p. s. i., and their average elongation, 3.7%. Again there is illustrated a positive and very substantial increase in both tensile strength and elongation as a result of the practice of the present method.

*Example 12.*—Parts were prepared of about 1.75% metallic manganese powder admixed with the balance of pure Swedish iron powder, pressed at 50,000 p. s. i., and thereafter sintered at 2000° F. The tensile strengths for the resulting parts, using different percentages (by volume) of hydrogen chloride with the balance hydrogen as a sintering atmosphere, are shown in the following table:

| Percent HCl in the Sintering Gas | Tensile Strength in p. s. i. |
|----------------------------------|------------------------------|
| 0                                | 3,970                        |
| 1                                | 5,000                        |
| 5                                | 7,240                        |
| 10                               | 11,570                       |

*Example 13.*—Parts were prepared of 0.25% molybdenum powder admixed with the balance of pure Swedish iron powder, pressed at 50,000 p. s. i., and thereafter sintered at 2000° F. The tensile strengths for the resulting parts, using different percentages (by volume) of hydrogen chloride with the balance hydrogen as a sintering atmosphere, are shown in the following table:

| Percent HCl in the Sintering Gas | Tensile Strength in p. s. i. |
|----------------------------------|------------------------------|
| 0                                | 7,780                        |
| 1                                | 11,720                       |
| 5                                | 13,330                       |
| 10                               | 15,930                       |

Further tests were made to illustrate the application of the present process to compositions having a substantially higher molybdenum content. In the first group of these

tests, compositions were made up with about 4% molybdenum and the balance iron. A group of test bars of this composition was sintered in pure hydrogen and then tested. These bars showed an average tensile strength of 18,100 p. s. i. and an average elongation of 3.9%. A similar group of test bars of the identical composition and mode of preparation was sintered in a gaseous atmosphere consisting essentially of about 5% hydrogen chloride and the balance hydrogen. These bars, when tested, showed an average tensile strength of 19,800 p. s. i. and an average elongation of 4.9%. In this instance it is noted that, while the average tensile strength is but little higher when following the practice of the present invention, the elongation found was substantially greater.

15 A further group of test bars with a still higher molybdenum content was prepared. In this instance the composition was about 8½% molybdenum with the balance iron. A group of such test bars was prepared and sintered in pure hydrogen and then tested, with the test results showing an average tensile strength of 19,030 p. s. i. and an average elongation of 5.8%. A similar group of test bars of the identical composition (about 8½% molybdenum and the balance iron) was sintered in an atmosphere consisting essentially of about 5% hydrogen chloride and the balance hydrogen. The bars of this group, when tested, showed an average tensile strength of 26,300 p. s. i. and an average elongation of 5.7%. In this instance it is noted that the elongation is substantially the same when using the process of the present invention as without it, but the tensile strength is very substantially enhanced. This example was prepared for the purpose of illustrating a high limit of molybdenum content to which the present invention is believed applicable.

25 *Example 14.*—Parts were prepared of 1.05% chromium powder admixed with the balance of pure Swedish iron powder, pressed at 50,000 p. s. i., and thereafter sintered at 2000° F. The tensile strengths for the resulting parts, using different percentages (by volume) 30 of hydrogen chloride with the balance hydrogen as a sintering atmosphere, are shown in the following table:

| Percent HCl in the Sintering Gas | Tensile Strength in p. s. i. |
|----------------------------------|------------------------------|
| 0                                | 4,650                        |
| 1                                | 6,520                        |
| 5                                | 12,120                       |
| 10                               | 9,530                        |

50 From the above, it will be noted that the maximum strength in iron-chrome parts is attained at a value under 10% hydrogen chloride in the atmosphere and closer to 5%, although the parts made and sintered in the 10% 55 hydrogen chloride atmosphere were about twice as strong as those sintered in an atmosphere of pure hydrogen.

Further tests have been made to illustrate the application of the process to compositions having substantially higher contents of chromium. In a first group 60 of these tests the starting composition was about 4% chromium and the balance iron (the chromium being added in the form of ferro-chromium having a 67.7% chromium content). A group of test bars of this composition was sintered in pure hydrogen and then tested with the test results showing a tensile strength (average) 65 of 5,170 p. s. i. and an elongation of 2.4%. A second group of test bars of the same composition was sintered in an atmosphere consisting essentially of 5% hydrogen chloride and the balance hydrogen and then tested. The test results in this instance showed an average tensile strength of 8,500 p. s. i. and an average elongation of 70 2.3%. Summarizing these results, it is noted that the practice of the present process resulted in very substantial enhancement of the tensile strength while the elongation remained substantially constant.

A further set of test bars was made up using a maximum limit of chromium for the present invention, i. e. about 28% chromium, with the balance iron (the chromium being added as aforesaid as a 67.7% ferro-chromium alloy). In this instance the average test results of a group of bars sintered in pure hydrogen was 2,260 p. s. i. as to tensile strength and 0.8% as to elongation; while a group of bars of the same composition, sintered in accordance with the present invention in an atmosphere consisting essentially of about 5% hydrogen chloride and the balance hydrogen, showed test results of 2,570 p. s. i. as to tensile strength and 2.0% as to elongation. Here it will be noted that, while the presence of chromium in substantial amounts appears to reduce the tensile strength under all circumstances, the practice of the present invention results in some substantial enhancement of the tensile strength and a very substantial enhancement in the elongation as contrasted with prior art practices involving sintering in pure hydrogen.

*Example 15.*—In view of the very desirable results in the increase of tensile strength for a number of binary alloys as herein given, it was thought that the present invention could be advantageously used on a material substantially equivalent in composition to a standard stainless steel. Such a composition was made up in powder form and was substantially 19% chromium, 1.6% manganese, 9% nickel and the balance iron. A series of test bars was made of this composition by pressing at 50,000 p. s. i. and then sintering in each instance at 2000° F. A first group of these test bars was sintered in pure hydrogen and showed an average tensile strength of 3,240 p. s. i. and an average elongation of 2.4%. A second group of test bars of this identical composition was made up in the same way and sintered as aforesaid in an atmosphere consisting essentially of 5% hydrogen chloride and the balance hydrogen. This group of bars, when tested, showed an average tensile strength of 5,600 p. s. i. and an average elongation of about 2.1%. Thus it is deemed that the process is applicable to multi-metal alloys such as stainless steels, wherein, however, the composition is within the limits herein set out for the several binary alloys, which have been made and tested as aforesaid. The fact that the elongation is slightly less for material produced by the present process is not considered prohibitive as it is well within tolerable limits.

*Example 16.*—The parts in this group were made up of 98% Swedish iron powder and 2% graphite, pressed at 60,000 p. s. i. and then sintered at various temperatures and under conditions as set forth in the following table:

| Atmosphere                   | Tempera-ture, ° F. | Tensile Strength (p. s. i.) |
|------------------------------|--------------------|-----------------------------|
| 100%, H <sub>2</sub>         | 1,800              | 12,500                      |
| 100%, H <sub>2</sub>         | 1,900              | 15,000                      |
| 100% H <sub>2</sub>          | 2,000              | 26,000                      |
| 90% H <sub>2</sub> , 10% HCl | 1,800              | 23,000                      |
| 90% H <sub>2</sub> , 10% HCl | 1,900              | 28,000                      |
| 90% H <sub>2</sub> , 10% HCl | 2,000              | 28,500                      |

These tests are deemed to indicate that iron-carbon alloys, simulating steel, follow the trend set forth in the application and show substantially increased tensile strengths when the process of the present invention is employed in connection with the sintering.

Further tests were made to illustrate the application of the process to even higher carbon contents in iron. To this end a group of samples was made up using "Swedish sponge" as a source of iron, this being a commercially available type of iron powder, and using carbon in each instance in the form of graphite. These tests employed a composition consisting essentially of about 4% carbon with the balance iron. All bars of this composition were found to be very brittle and to have a very low, and in effect insignificant, elongation. For this reason no data as to elongation are given. The bars were all made by

pressing the composition at 60,000 p. s. i. and sintering at 2000° F. for one hour. A group of three such bars, when sintered in pure hydrogen, was found to have an average tensile strength of about 28,650 p. s. i. Another group of three such bars was prepared as aforesaid of the identical composition and mode of preparation and sintered in an atmosphere consisting essentially of 10% hydrogen chloride and the balance hydrogen. This group was found to have an average tensile strength of 32,470 p. s. i. It is believed, however, that about 4% is the maximum carbon content which is reasonably tolerable in a ferrous base alloy as aforesaid. Such an alloy in all instances in this case is considered to be one having a substantial preponderance of iron, i. e. substantially over 50% even in instances where quite large percentages of alloying constituents are present, such as stainless steel.

While the process of the present invention has been disclosed as applied to a limited number of the many possible combinations to which it is applicable, the principles herein set forth are applicable generally within the limits stated. It is intended that the appended claims shall be construed to cover all reasonable equivalents as will occur to those skilled in the art from the foregoing particular disclosure, and that the claims should be construed validly as broadly as the state of the prior art permits.

What is claimed is:

1. The process of making metallic parts starting with a metallic material consisting essentially of at least one of the relatively difficultly chloridizable metallic powders selected from the group which consists of (a) the metals: iron, copper, nickel and cobalt and mixtures and alloys consisting essentially of at least two of said metals, (b) mixtures and alloys corresponding generally to bronze and consisting essentially of up to about 10% tin and the balance copper, (c) mixtures and alloys corresponding generally in composition to ferrous base alloys and consisting essentially of:

up to about 4% carbon,  
up to about 20% tungsten,  
up to about 1.75% manganese,  
up to about 28% chromium,  
up to about 8½% molybdenum,

and the balance in any such composition iron, wherein iron is present in a predominant amount; said process comprising the steps of compacting a predetermined amount of said material by mechanical pressure to form it into a green pressed blank having a shape and size predetermined in accordance with the shape and size of the part to be made, and thereafter heat treating said green pressed blank in a non-oxidizing atmosphere containing at least about 0.1% of gaseous hydrogen chloride by volume, and wherein said hydrogen chloride is introduced into said atmosphere from a source separate and independent of any chloride which may be present in admixture in said metallic material, by raising the temperature of said material of said blank to a point at which at least one metal present is brought to the point of incipient fusion in said atmosphere, and by supplying hydrogen chloride gas to said atmosphere from a source independent of the material making up the parts being treated.

2. The process in accordance with claim 1, wherein the volume concentration of gaseous hydrogen chloride in said atmosphere is about 0.5% to about 10%.

3. The process in accordance with claim 1, wherein the volume concentration of gaseous hydrogen chloride in said atmosphere is about 5% to about 15%.

4. The process in accordance with claim 1, wherein said non-oxidizing atmosphere also contains hydrogen.

5. The process in accordance with claim 1, wherein said non-oxidizing atmosphere consists essentially of a mixture of gaseous hydrogen chloride and hydrogen.

6. The process in accordance with claim 1, wherein

said heat treating is carried on at substantially the same temperature at which some one metal present in said metallic material will sinter in the same atmosphere without hydrogen chloride present therein, so as to produce a part having enhanced physical properties in respect to the corresponding physical properties of such a part sintered in the same atmosphere but without hydrogen chloride therein.

7. The process in accordance with claim 1, wherein said heat treating is carried on at a temperature substantially below that temperature at which some one metal present in said metallic material will sinter in the same atmosphere in the absence of hydrogen chloride therein, so as to produce a part having substantially as desirable physical properties as the part would have if sintered in the same atmosphere in the absence of hydrogen chloride therein at the temperature at which some metal present will sinter in the absence of hydrogen chloride.

8. The process in accordance with claim 1, wherein said heat treating is carried on at a temperature somewhat lower than that at which some one metal present in said metallic material will sinter in the same atmosphere in the absence of hydrogen chloride therein, so as to produce a part having somewhat enhanced physical properties in respect to the properties which would be present in a similar part sintered in the same atmosphere in the absence of hydrogen chloride at the temperature at which this metallic material would sinter in such atmosphere in which hydrogen chloride was absent.

9. The process in accordance with claim 1, wherein said metallic material used in forming the metallic parts to be treated is substantially free of all intermixed chlorides, whereby all the hydrogen chloride present in said non-oxidizing atmosphere is supplied thereto from a source external of the parts being sintered.

10. The process in accordance with claim 1, wherein said metallic material consists essentially of iron and copper and wherein said atmosphere contains from about 5% to about 15% hydrogen chloride by volume, the temperature of the heat treatment being at least that at which copper powder is brought to the point of incipient fusion.

11. The process in accordance with claim 1, wherein said metallic material consists essentially of up to about 4% carbon and the balance iron, and wherein said atmosphere contains from about 5% to about 15% gaseous hydrogen chloride by volume.

12. The process in accordance with claim 1, wherein said metallic material consists essentially of metallic iron, and wherein said atmosphere contains from about 5% to about 15% gaseous hydrogen chloride by volume,

13. The process in accordance with claim 1, wherein said metallic material consists essentially of iron and nickel, and wherein said atmosphere contains from about 5% to about 15% gaseous hydrogen chloride by volume, the temperature of the heat treatment being at least that at which nickel powder is brought to the point of incipient fusion.

14. The process in accordance with claim 1, wherein said metallic material consists essentially of up to about 10% tin and the balance copper, and wherein said atmosphere contains from about 5% to about 15% gaseous hydrogen chloride by volume, the temperature of the heat treatment being at least that at which tin powder is brought to the point of incipient fusion.

15. The process in accordance with claim 1, wherein said heat treatment was carried on for a time period substantially less than that in which a part of the same composition would be sintered in the same atmosphere without hydrogen chloride present therein, so as to provide for increased production of sintered parts having at least as good physical properties as would be provided if such parts were sintered for the conventional time in the same atmosphere without hydrogen chloride present therein.

20 16. The process in accordance with claim 1, wherein said heat treatment is carried on at substantially the same temperature at which a part having the same composition would be sintered in the same atmosphere but without hydrogen chloride present therein, and for a time period substantially less than has been conventional for sintering such a part in such an atmosphere but without hydrogen chloride, so as to provide for increased production of sintered parts each having at least as good physical properties as would be produced from the same unsintered parts if sintered in the same atmosphere at the same temperature but without hydrogen chloride present.

25 17. The process in accordance with claim 1, wherein the heat treating step aforesaid is carried on in a sintering zone, wherein said non-oxidizing atmosphere is maintained in said sintering zone by substantially continuously passing through said zone a non-oxidizing gaseous medium including at least 0.1% (by volume) gaseous hydrogen chloride as aforesaid, and wherein said gaseous hydrogen chloride is supplied to said gaseous medium from a source external of said sintering zone and also external of the green pressed blanks introduced into said zone for heat treatment therein.

No references cited.